



US008480808B2

(12) **United States Patent**  
**Olson et al.**

(10) **Patent No.:** **US 8,480,808 B2**  
(b5) **Date of Patent:** **\*Jul. 9, 2013**

(54) **DETERGENT COMPOSITIONS WITH  
COMBINATIONS OF ACRYLIC AND MALEIC  
ACID HOMOPOLYMERS AND/OR SALTS  
THEREOF FOR ALUMINUM PROTECTION**

(75) Inventors: **Erik Christian Olson**, Savage, MN  
(US); **Devon Beau Hammel**,  
Minneapolis, MN (US)

(73) Assignee: **Ecolab USA Inc.**, Saint Paul, MN (US)

(\*) Notice: Subject to any disclaimer, the term of this patent is extended or adjusted under 35 U.S.C. 154(b) by 0 days.

This patent is subject to a terminal disclaimer.

(21) Appl. No.: **13/562,695**

(22) Filed: **Jul. 31, 2012**

(65) **Prior Publication Data**

US 2012/0295830 A1 Nov. 22, 2012

**Related U.S. Application Data**

(63) Continuation of application No. 12/869,804, filed on Aug. 27, 2010, now Pat. No. 8,263,540.

(51) **Int. Cl.**

**B08B 3/04** (2006.01)  
**C11D 1/00** (2006.01)  
**C11D 3/08** (2006.01)  
**C11D 3/37** (2006.01)

(52) **U.S. Cl.**

USPC ..... **134/2**; 134/41; 134/42; 510/245;  
510/267; 510/434; 510/466; 510/476; 510/477

(58) **Field of Classification Search**

USPC ..... 510/245, 267, 434, 466, 476, 477; 134/2,  
134/41, 42

See application file for complete search history.

(56) **References Cited**

**U.S. PATENT DOCUMENTS**

|              |         |                 |
|--------------|---------|-----------------|
| 601,723 A    | 4/1898  | Werts           |
| 4,834,955 A  | 5/1989  | Mouche et al.   |
| 5,320,771 A  | 6/1994  | Turcotte et al. |
| 5,389,276 A  | 2/1995  | Coffey et al.   |
| 5,431,847 A  | 7/1995  | Winston et al.  |
| 5,510,048 A  | 4/1996  | Durbut et al.   |
| 6,686,325 B2 | 2/2004  | Hoyt et al.     |
| 6,812,194 B2 | 11/2004 | Ruhr et al.     |
| 7,524,535 B2 | 4/2009  | Kim et al.      |
| 7,524,803 B2 | 4/2009  | Lentsch et al.  |
| 7,601,280 B2 | 10/2009 | Kinlen          |
| 7,601,425 B2 | 10/2009 | Stoffer et al.  |
| 7,638,473 B2 | 12/2009 | Smith et al.    |
| 7,655,279 B2 | 2/2010  | Dietsche et al. |

|                   |         |                              |
|-------------------|---------|------------------------------|
| 7,662,241 B2      | 2/2010  | Sinko                        |
| 7,727,420 B2      | 6/2010  | Ward                         |
| 8,263,540 B2 *    | 9/2012  | Olson et al. .... 510/245    |
| 2003/0109394 A1   | 6/2003  | Ruhr et al.                  |
| 2003/0176305 A1   | 9/2003  | Hoyt et al.                  |
| 2008/0233390 A1   | 9/2008  | Gothlich et al.              |
| 2008/0287335 A1   | 11/2008 | Smith                        |
| 2009/0029155 A1   | 1/2009  | Gothlich et al.              |
| 2009/0176685 A1   | 7/2009  | Ward                         |
| 2010/0298193 A1 * | 11/2010 | Tjelta et al. .... 510/224   |
| 2010/0300493 A1 * | 12/2010 | Snodgrass et al. .... 134/26 |

**FOREIGN PATENT DOCUMENTS**

|    |                   |        |
|----|-------------------|--------|
| WO | WO 01/05931 A1    | 1/2001 |
| WO | WO 2004/020562 A1 | 3/2004 |

**OTHER PUBLICATIONS**

“ACUMERT™ 1510 Polyacrylic Acid Homopolymer”, [http://www.rohahaas.com/wcm/products/product\\_detail.page?product=1121949&display=...](http://www.rohahaas.com/wcm/products/product_detail.page?product=1121949&display=...) DOW, printed Internet May 10, 2010, 2 pages.

Amin, Mohammed A. et al., “Polyacrylic acid as a corrosion inhibitor for aluminium in weakly alkaline solutions. Part I: Weight loss, polarization, impedance EFM and EDX studies”, *Corrosion Science* 51 (2009) 658-667.

Kelien Water Treatment Chemicals, “Maleic acid/acrylic acid copolymer (MA/AA)”, <http://www.kelien.com/products/MA-AA%20COPOLYMER.htm>, printed Internet May 10, 2010, 1 page.

Akzo Nobel Surface Chemistry LLC, “Technical Information Surface Chemistry” Aquatreat® Products Polymer Selection Guide, <http://surface.akzonobel.com>, 2009, 3 pages.

Rohm and Haas, “ACUSOL™ 445/445N/445ND Detergent Polymer for Laundry”, 3 pages, 2008.

Rohm and Haas, “ACUMERT™ 1510 Polyacrylic Acid Homopolymer”, 3 pages, 2008.

Waterfront™ Product Information, BWA Water Additives, Belclene® 200—the industry Standard Antiscalant for Calcium Carbonate Control in Severe Service Conditions, [www.wateradditives.com](http://www.wateradditives.com), 2006, 2 pages.

Ecolab USA Inc. et al., PCT/IB2011/053741, filed Aug. 25, 2011, “Notification of Transmittal of the International Search Report and The Written Opinion of the International Searching Authority” mailed May 30, 2012.

\* cited by examiner

*Primary Examiner* — Brian P Mruk

(74) *Attorney, Agent, or Firm* — McKee, Voorhees & Sease, P.L.C.

(57) **ABSTRACT**

A warewashing detergent composition is provided for use for in cleaning of alkaline sensitive metals such as aluminum or aluminum containing alloys. The compositions include alternatives to sodium tripolyphosphate and/or other phosphorous containing raw materials, while retaining cleaning performance and corrosion prevention. According to the invention, a synergistic combination of polyacrylic and polymaleic polymers is used as corrosion inhibitors in traditional alkaline detergent compositions.

**20 Claims, No Drawings**

## 1

**DETERGENT COMPOSITIONS WITH  
COMBINATIONS OF ACRYLIC AND MALEIC  
ACID HOMOPOLYMERS AND/OR SALTS  
THEREOF FOR ALUMINUM PROTECTION**

**CROSS-REFERENCE TO RELATED  
APPLICATIONS**

This application is a Continuation Application of U.S. Ser. No. 12/869,804 filed Aug. 27, 2010, now U.S. Pat. No. 8,263,540 issued on Sep. 11, 2012, herein incorporated by reference in its entirety.

**FIELD OF THE INVENTION**

The invention relates to detergent and cleaning compositions, particularly warewashing compositions comprising acrylic and maleic acid (or salts thereof) homopolymers, and their use for cleaning of alkaline sensitive metals such as aluminum or aluminum containing alloys.

**BACKGROUND OF THE INVENTION**

In recent years there has been an ever increasing trend towards safer and sustainable detergent compositions. This has led to the development of alternative complexing agents, builders, threshold agents, corrosion inhibitors, and the like, which are used instead of predominantly phosphorous containing compounds. Phosphates can bind calcium and magnesium ions, provide alkalinity, act as threshold agents, and protect alkaline sensitive metals such as aluminum and aluminum containing alloys.

Other corrosion inhibitors include silicates, such as, sodium silicate. Sodium silicate has a tendency to begin precipitating from aqueous solution at a pH below 11, thus reducing its effectiveness to prevent corrosion of the contacted surfaces when used in cleaning solutions having a lower pH. Additionally, when allowed to dry on a surface silicates form films and/or spots which are visible and they are very difficult to remove. The presence of these silicon containing deposits can affect the texture, appearance, and on cooking or storage surfaces the taste of the materials that come into contact with the cleaned surfaces.

It is an object of the invention to address at least one of the above problems and/or to offer detergent compositions with usage and/or environmental benefits.

**SUMMARY OF THE INVENTION**

In one embodiment, the present invention relates to a corrosion inhibiting composition that may be used in formulation of detergents, cleaning compositions, and in protecting aluminum and aluminum containing alloys from corrosion. The corrosion inhibiting composition comprises a mixture of polyacrylic and polymaleic acid homopolymers (or salts thereof) in a synergistic ratio. The combination of polyacrylic acid to polymaleic acid homopolymers (or salt thereof), is preferably a ratio of at least about 1:1 (wt %). In a more preferred embodiment the ratio is about 2:1 (wt %) and in a most preferred embodiment the ratio is about 7:3 (wt %).

In one embodiment a detergent composition is provided according to the invention. A detergent composition including an alkalinity source and a combination of polyacrylic acid and polymaleic acid homopolymers (or salts thereof) for corrosion inhibition. The cleaning agent also preferably includes a detergents amount of a surfactant. The alkaline source can be provided in an amount effective to provide a use composition

## 2

having a pH of at least about 8. The combination of polyacrylic acid and polymaleic acid homopolymers (or salts thereof) is provided in an amount sufficient to reduce corrosion of aluminum and/or aluminum containing alloys at a pH of about 8 or greater.

Articles which require such cleaning according to the invention includes any article with a surface that contains an alkaline sensitive metal, such as, aluminum or aluminum containing alloys. Such articles can be found in industrial plants, maintenance and repair services, manufacturing facilities, kitchens, and restaurants. Exemplary equipment having a surface containing an alkaline sensitive metals include sinks, cookware, utensils, machine parts, vehicles, tanker trucks, vehicle wheels, work surfaces, tanks, immersion vessels, spray washers, and ultrasonic baths. In addition, a detergent composition is provided according to the invention that can be used in environments other than inside a dishwashing machine. Alkaline sensitive metals in need of cleaning are found in several locations. Exemplary locations also include trucks, vehicle wheels, ware, and facilities. One exemplary application of the alkaline sensitive metal cleaning detergent composition for cleaning alkaline sensitive metals can be found in cleaning vehicle wheels in a vehicle washing facility. Compositions of the invention may be used in any of these applications and the like.

The invention also includes methods for cleaning aluminum and/or aluminum containing alloys by contacting the surface of the same with the detergent/cleaning compositions of the invention. The detergent/cleaning compositions include the corrosion inhibiting composition of a synergistic mixture of polyacrylic acid and polymaleic acid homopolymers or salts thereof.

The invention also includes methods for protecting aluminum and/or aluminum containing alloys from corrosion by use of the novel corrosion inhibiting composition of the invention. The method involves the step of contacting the surface of aluminum, or an aluminum containing alloy with the corrosion inhibiting composition of the invention. The novel corrosion inhibiting composition includes a synergistic mixture of polyacrylic acid and polymaleic acid homopolymers or salts thereof.

Also included is a method for manufacturing a detergent composition. The method can include a step of adding a corrosion inhibitor comprising a combination of polyacrylic acid and polymaleic acid homopolymers (or salts thereof) to a detergent composition. The corrosion inhibitor can be added to the detergent composition when the detergent composition is a concentrate and/or when the detergent composition is a use solution.

**DETAILED DESCRIPTION OF THE INVENTION**

In this specification and the claims that follow, reference will be made to a number of terms that shall be defined to have the following meanings:

The phrase "alkaline sensitive metal" identifies those metals that exhibit corrosion and/or discoloration when exposed to an alkaline detergent in solution. An alkaline solution is an aqueous solution having a pH that is greater than 8. Exemplary alkaline sensitive metals include soft metals such as aluminum, nickel, tin, zinc, copper, brass, bronze, and mixtures thereof. Aluminum and aluminum alloys are common alkaline sensitive metals that can be cleaned by the warewash detergent compositions of the invention.

As used herein, weight percent (wt-%), percent by weight, % by weight, and the like are synonyms that refer to the

concentration of a substance as the weight of that substance divided by the total weight of the composition and multiplied by 100.

As used herein, the term "about" modifying the quantity of a component or ingredient in the compositions of the invention or employed in the methods of the invention refers to variation in the numerical quantity that can occur, for example, through typical measuring and liquid handling procedures used for making concentrates or use solutions in the real world; through inadvertent error in these procedures; through differences in the manufacture, source, or purity of the ingredients employed to make the compositions or carry out the methods; and the like. The term about also encompasses amounts that differ due to different equilibrium conditions for a composition resulting from a particular initial mixture. Whether or not modified by the term "about," the claims include equivalents to the quantities.

The term "surfactant" or "surface active agent" refers to an organic chemical that when added to a liquid changes the properties of that liquid at a surface.

"Cleaning" means to perform or aid in soil removal, bleaching, de-scaling, de-staining, microbial population reduction, rinsing, or combination thereof.

As used herein, the term "substantially free" refers to compositions completely lacking the component or having such a small amount of the component that the component does not affect the performance of the composition. The component may be present as an impurity or as a contaminant and shall be less than 0.5 wt. %. In another embodiment, the amount of the component is less than 0.1 wt-% and in yet another embodiment, the amount of component is less than 0.01 wt. %.

As used herein, the term "ware" includes items such as eating and cooking utensils. As used herein, the term "ware-washing" refers to washing, cleaning, or rinsing ware.

As used herein, a solid cleaning composition refers to a cleaning composition in the form of a solid such as a powder, a particle, an agglomerate, a flake, a granule, a pellet, a tablet, a lozenge, a puck, a briquette, a brick, a solid block, a unit dose, or another solid form known to those of skill in the art. The term "solid" refers to the state of the detergent composition under the expected conditions of storage and use of the solid detergent composition. In general, it is expected that the detergent composition will remain in solid form when exposed to elevated temperatures of 100° F. and preferably 120° F. A cast, pressed, or extruded "solid" may take any form including a block. When referring to a cast, pressed, or extruded solid it is meant that the hardened composition will not flow perceptibly and will substantially retain its shape under moderate stress, pressure, or mere gravity. For example, the shape of a mold when removed from the mold, the shape of an article as formed upon extrusion from an extruder, and the like. The degree of hardness of the solid cast composition can range from that of a fused solid block, which is relatively dense and hard similar to concrete, to a consistency characterized as being malleable and sponge-like, similar to caulking material.

It should be noted that, as used in this specification and the appended claims, the singular forms "a," "an," and "the" include plural referents unless the content clearly dictates otherwise. Thus, for example, reference to a composition containing "a compound" includes a mixture of two or more compounds. It should also be noted that the term "or" is generally employed in its sense including "and/or" unless the content clearly dictates otherwise.

The term "actives" or "percent actives" or "percent by weight actives" or "actives concentration" are used interchangeably herein and refers to the concentration of those

ingredients involved in cleaning expressed as a percentage minus inert ingredients such as water or salts.

As used herein, the terms "sodium tripolyphosphate-free" or "STPP-free" refers to a composition, mixture, or ingredients that do not contain tripolyphosphates or to which the same has not been added. Should sodium tripolyphosphate or other phosphate containing compounds be present through contamination of a composition, mixture, or ingredients, the amount of the same shall be less than 0.5 wt. %. In a preferred embodiment, the amount of the same is less than 0.1 wt-% and in more preferred embodiment, the amount is less than 0.01 wt. %.

The term "substantially similar cleaning performance" refers generally to achievement by a substitute cleaning product or substitute cleaning system of generally the same degree (or at least not a significantly lesser degree) of cleanliness or with generally the same expenditure (or at least not a significantly lesser expenditure) of effort, or both.

Many articles having a surface that requires cleaning contain an alkaline sensitive metal, such as, aluminum or aluminum containing alloys. Such articles can be found in industrial plants, maintenance and repair services, manufacturing facilities, kitchens, and restaurants. Exemplary equipment having a surface containing an alkaline sensitive metals include sinks, cookware, utensils, machine parts, vehicles, tanker trucks, vehicle wheels, work surfaces, tanks, immersion vessels, spray washers, and ultrasonic baths. In addition, a warewash detergent composition is provided according to the invention that can be used in environments other than inside a dishwashing machine. Alkaline sensitive metals in need of cleaning are found in several locations. Exemplary locations also include trucks, vehicle wheels, ware, and facilities. One exemplary application of the alkaline sensitive metal cleaning/warewash detergent composition for cleaning alkaline sensitive metals can be found in cleaning vehicle wheels in a vehicle washing facility. Compositions of the invention may be used in any of these applications.

According to the invention a detergent composition is provided comprising an alkaline source and a novel corrosion inhibitor comprising a combination of polyacrylic and polymaleic acid homopolymers (or salts thereof). The combination of polyacrylic acid homopolymer (or salts thereof) to polymaleic acid homopolymer (or salt thereof), is preferably a ratio of at least about 1:1 (wt %). In a preferred embodiment the ratio is about 2:1 (wt %) and in a most preferred embodiment the ratio is about 7:3 (wt %).

The composition may also preferably include a detergents amount of a surfactant. The alkaline source can be provided in an amount effective to provide a use composition having a pH of at least about 8. The corrosion inhibitor is provided in an amount sufficient to reduce corrosion of aluminum when the detergent composition is provided as a use composition for washing aluminum and aluminum containing alloys.

The detergent composition can be made available as multiple concentrates that are diluted and combined at the situs of use to provide a use solution for application to alkaline sensitive metals. An advantage of providing concentrates that are later combined is that shipping and storage costs can be reduced because it can be less expensive to ship and store a concentrate rather than a use solution and is also more sustainable because less packaging is used. Although the detergent composition according to the invention can be provided as multiple concentrates, it should be understood that the composition can be provided as a ready to use solution. In addition, the multiple concentrates can include two or more

concentrates that are added together. In addition, the concentrates can be provided in the form of a liquid, solid, paste, gel, granulate, or powder.

The cleaning composition can be characterized as including an alkaline component and a corrosion inhibitor component. The alkaline component includes a source of alkalinity. The source of alkalinity is provided so that the use solution has a pH of at least 8.0. The corrosion inhibitor component includes a corrosion inhibitor of polyacrylic acid and polymaleic acid homopolymers (or salts thereof). The corrosion inhibitor component is provided for reducing corrosion of alkaline sensitive metals by the use solution having a pH of at least 8.0.

A surfactant component may also be present. The surfactant component provides cleaning properties when used as part of the use solution at a pH of at least 8.0. A threshold inhibitor/crystal modifier can also be provided to prevent calcium carbonate precipitation in a use solution provided at a pH in the range of 8.0 to 14.0. Further additional components include the use of chelants as discussed hereinafter.

#### Source of Alkalinity

The source of alkalinity can be any source of alkalinity that is compatible with the other components of the detergent composition and that will provide a use solution with the desired pH. Exemplary sources of alkalinity include alkali metal hydroxides, alkali metal salts, silicates, phosphates, amines, and mixtures thereof. Exemplary alkali metal hydroxides include sodium hydroxide, potassium hydroxide, and lithium hydroxide. The alkali metal hydroxide may be added to the composition in a variety of forms, including for example in the form of solid beads, dissolved in an aqueous solution, or a combination thereof. Alkali metal hydroxides are commercially available as a solid in the form of prilled solids or beads having a mix of particle sizes ranging from about 12-100 U.S. mesh, or as an aqueous solution, as for example, as a 45 wt. %, 50 wt. % and a 73 wt. % solution.

Exemplary alkali metal salts include sodium carbonate, trisodium phosphate, potassium carbonate, and mixtures thereof. Exemplary silicates include sodium metasilicates, sesquisilicates, orthosilicates, potassium silicates, and mixtures thereof. Exemplary phosphates include sodium pyrophosphate, potassium pyrophosphate, and mixtures thereof. Exemplary amines include alkanolamine. Exemplary alkanolamines include triethanolamine, monoethanolamine, diethanolamine, and mixtures thereof.

The source of alkalinity is provided in an amount sufficient to provide the use solution with a pH of at least 8.0. The use solution pH range is preferably between about 8.0 and about 13.0, and more preferably between 10.0 to 12.5. In general, the amount of alkalinity provided in the concentrate can be in an amount of at least about 0.05 wt. % based on the weight of the alkaline concentrate. The source of alkalinity in the concentrate is preferably between about 0.05 wt. % and about 99 wt. %, more preferably is between about 0.1 wt. % and about 95 wt. %, and most preferably is between 0.5 wt % and 90 wt %.

#### Corrosion Inhibitor Component

The invention comprises a novel corrosion inhibitor component of a mixture of polyacrylic acid and polymaleic acid (or salts thereof) homopolymers. The corrosion inhibitor component effectively reduces corrosion to alkaline sensitive metals such as aluminum or aluminum containing alloys at a pH of about 8 or greater. Preferred ratios of polyacrylic homopolymer to polymaleic homopolymer is about 1:1 (weight %). More preferably the ratio of polyacrylic homopolymer to polymaleic homopolymer is about 2:1 (weight %) and most preferably the ratio is about 7:3.

Polymaleic acid ( $C_4H_2O_3$ ) $x$  or hydrolyzed polymaleic anhydride or cis-2-butenedioic acid homopolymer, has the structural formula:



10 where n and m are any integer.

15 Examples of polymaleic homopolymers which may be used for the invention and that are particularly preferred are those with a molecular weight of about 200-2000. Commercially available polymaleic homopolymers include the Belclene 200 series of maleic acid homopolymers from BWA™ Water Additives, 979 Lakeside Parkway, Suite 925 Tucker, Ga. 30084, USA. Particularly preferred is Belclene 200 or Aquatreat AR-801 available from AkzoNobel.

20 Polyacrylic acids,  $(C_3H_4O_2)_n$  or 2-Propenoic acid homopolymer; Acrylic acid polymer; Poly(acrylic acid); Propenoic acid polymer; PAA have the following structural formula:



30 where n is any integer.

35 Examples of polyacrylic homopolymers which may be used for the invention are those with a molecular weight of at least about 4500. One source of commercially available polyacrylic homopolymers useful for the invention includes the 40 Acusol 445 series from The Dow Chemical Company, Wilmington Del., USA. Other polyacrylic acid homopolymers (and salts thereof) commercially available are Acusol 929 (10,000 MW) and Acumer 1510 (60,000 MW) both also available from Dow Chemical. Yet another commercially 45 available polyacrylic homopolymer is AQUATREAT AR-6 (100,000 MW) from AkzoNobel Strawinskyalaan 2555 1077 ZZ Amsterdam Postbus 75730 1070 AS Amsterdam.

The corrosion inhibitor component can be provided in the corrosion inhibitor concentrate in an amount sufficient to 50 provide a desired level of corrosion inhibition when used in the use solution. There should be sufficient amount of corrosion inhibitor to provide the desired corrosion inhibiting affect. It is expected that the upper limit on the corrosion inhibitor component will be controlled by solubility. The corrosion inhibitor component can be provided in the corrosion inhibitor concentrate in an amount of at least about 0.005 wt. %. It is preferred that the corrosion inhibitor component be provided in the concentrate in an amount between about 0.5 wt. % and about 50 wt. %, more preferably between about 55 1 wt. % and about 30 wt. %, and most preferably between 5% and 15% active.

#### Cleaning Agent/Surfactant

60 The detergent composition can include at least one cleaning agent comprising a surfactant or surfactant system. A variety of surfactants can be used in a warewashing composition, such as anionic, nonionic, cationic, and zwitterionic surfactants. It should be understood that surfactants are an

optional component of the detergent composition and can be excluded. The detergent composition, when provided as a concentrate, can include the cleaning agent in a range of between about 0.5 wt. % and about 20 wt. %, more preferably in a range between about 1 wt. % and 10 wt. %, and most preferably in a range between about 1.5 wt. % and 5 wt. %. Additional exemplary ranges of surfactant in a concentrate include about 0.05 wt. % to 7.5 wt. %, more preferably about 0.5 wt. % to 5 wt. %, and most preferably about 1 wt. % to 3 wt. %.

Exemplary surfactants that can be used are commercially available from a number of sources. For a discussion of surfactants, see Kirk-Othmer, Encyclopedia of Chemical Technology, Third Edition, volume 8, pages 900-912. When the composition includes a cleaning agent, the cleaning agent can be provided in an amount effective to provide a desired level of cleaning.

Anionic surfactants useful in detergent compositions include, for example, carboxylates such as alkylcarboxylates (carboxylic acid salts) and polyalkoxycarboxylates, alcohol ethoxylate carboxylates, nonylphenol ethoxylate carboxylates, and the like; sulfonates such as alkylsulfonates, alkylbenzenesulfonates, alkylarylsulfonates, sulfonated fatty acid esters, and the like; sulfates such as sulfated alcohols, sulfated alcohol ethoxylates, sulfated alkylphenols, alkylsulfates, sulfosuccinates, alkylether sulfates, and the like; and phosphate esters such as alkylphosphate esters, and the like. Exemplary anionic surfactants include sodium alkylarylsulfonate, alphaolefinsulfonate, and fatty alcohol sulfates.

Nonionic surfactants useful in the detergent composition include, for example, those having a polyalkylene oxide polymer as a portion of the surfactant molecule. Such nonionic surfactants include, for example, chlorine-, benzyl-, methyl-, ethyl-, propyl-, butyl- and other like alkyl-capped polyethylene glycol ethers of fatty alcohols; polyalkylene oxide free nonionics such as alkyl polyglycosides; sorbitan and sucrose esters and their ethoxylates; alkoxylated ethylene diamine; alcohol alkoxylates such as alcohol ethoxylate propoxylates, alcohol propoxylates, alcohol propoxylate ethoxylate propoxylates, alcohol ethoxylate butoxylates, and the like; nonylphenol ethoxylate, polyoxyethylene glycol ethers and the like; carboxylic acid esters such as glycerol esters, polyoxyethylene esters, ethoxylated and glycol esters of fatty acids, and the like; carboxylic amides such as diethanolamine condensates, monoalkanolamine condensates, polyoxyethylene fatty acid amides, and the like; and polyalkylene oxide block copolymers including an ethylene oxide/propylene oxide block copolymer such as those commercially available under the trademark PLURONIC® (BASF-Wyandotte), and the like; and other like nonionic compounds. Silicone surfactants such as the ABIL® B8852 can also be used.

Cationic surfactants that can be used in the detergent composition include amines such as primary, secondary and tertiary monoamines with C<sub>1-8</sub> alkyl or alkenyl chains, ethoxylated alkylamines, alkoxylates of ethylenediamine, imidazoles such as a 1-(2-hydroxyethyl)-2-imidazoline, a 2-alkyl-1-(2-hydroxyethyl)-2-imidazoline, and the like; and quaternary ammonium salts, as for example, alkylquaternary ammonium chloride surfactants such as n-alkyl(C<sub>12</sub>-C<sub>18</sub>) dimethylbenzyl ammonium chloride, n-tetradecyldimethylbenzylammonium chloride monohydrate, a naphthylene-substituted quaternary ammonium chloride such as dimethyl-1-naphthylmethylammonium chloride, and the like. The cationic surfactant can be used to provide sanitizing properties.

Zwitterionic surfactants that can be used in the detergent composition include betaines, imidazolines, and propionates.

If the detergent composition is intended to be used in an automatic dishwashing or warewashing machine, the surfactants selected, if any surfactant is used, can be those that provide an acceptable level of foaming. It should be understood that warewashing compositions for use in automatic dishwashing or warewashing machines are generally considered to be low-foaming compositions.

The surfactant can be selected to provide low foaming properties. One would understand that low foaming surfactants that provide the desired level of detergative activity are advantageous in an environment such as a dishwashing machine where the presence of large amounts of foaming can be problematic. In addition to selecting low foaming surfactants, one would understand that defoaming agents can be utilized to reduce the generation of foam. Accordingly, surfactants that are considered low foaming surfactants as well as other surfactants can be used in the detergent composition and the level of foaming can be controlled by the addition of a defoaming agent.

#### 20 Threshold Agent/Crystal Modifier Component

The detergent composition may also include a threshold agent or crystal modifier for reducing precipitation of calcium carbonate in the use solution. In general, it is expected that the threshold agent/crystal modifier component will loosely hold calcium to reduce precipitation of calcium carbonate once it is subjected to a pH of at least 8.0.

Exemplary threshold agents/crystal modifiers include phosphonocarboxylic acids, phosphonates, phosphates, chelants, polymers, and mixtures thereof. Exemplary phosphonocarboxylic acids include those available under the name Bayhibit™ AM from Bayer, and include 2-phosphonobutane-1,2,4, tricarboxylic acid (PBTC). Exemplary phosphonates include amino tri(methylene phosphonic acid), 1-hydroxy ethylidene 1,1-diphosphonic acid, ethylene diamine tetra(methylene phosphonic acid), hexamethylene diamine tetra(methylene phosphonic acid), diethylene triamine penta(methylene phosphonic acid), and mixtures thereof. Exemplary phosphonates are available under the name Dequest™ from Monsanto. Exemplary polymers include polyacrylates, polymethacrylates, polyacrylic acid, polyitaconic acid, polymaleic acid, sulfonated polymers, copolymers and mixtures thereof. It should be understood that the mixtures can include mixtures of different acid substituted polymers within the same general class. In addition, it should be understood that salts of acid substituted polymers can be used. The useful carboxylated polymers may be generically categorized as water-soluble carboxylic acid polymers such as polyacrylic and polymethacrylic acids or vinyl addition polymers, in addition to the acid-substituted polymers used in the present invention. Of the vinyl addition polymers contemplated, maleic anhydride copolymers as with vinyl acetate, styrene, ethylene, isobutylene, acrylic acid and vinyl ethers are examples. The polymers tend to be water-soluble or at least colloidally dispersible in water. The molecular weight of these polymers may vary over a broad range although it is preferred to use polymers having average molecular weights ranging between 1,000 up to 1,000,000, more preferably a molecular weight of 100,000 or less, and most preferably a molecular weight between 1,000 and 10,000.

The polymers or copolymers (either the acid-substituted polymers or other added polymers) may be prepared by either addition or hydrolytic techniques. Thus, maleic anhydride copolymers are prepared by the addition polymerization of maleic anhydride and another comonomer such as styrene. The low molecular weight acrylic acid polymers may be prepared by addition polymerization of acrylic acid or its salts

either with itself or other vinyl comonomers. Alternatively, such polymers may be prepared by the alkaline hydrolysis of low molecular weight acrylonitrile homopolymers or copolymers. For such a preparative technique see Newman U.S. Pat. No. 3,419,502.

The threshold agent/crystal modifier component should be provided in an amount sufficient so that when it is in the use solution it sufficiently disrupts crystal growth or prevents the precipitation of calcium carbonate and other insoluble salts such as magnesium silicate, magnesium hydroxide, and the like. In a preferred embodiment the threshold agent/crystal modifier component can be provided in a range of about 0.0001 wt. % to about 25 wt. %, more preferably in a range between about 0.001 wt. % and about 10 wt. %, and most preferably between about 0.01% and 8% based on the weight of the concentrate. It should be understood that the polymers, phosphonocarboxylates, and phosphonates can be used alone or in combination.

#### Hydrotrope Component

A hydrotrope component can be used to help stabilize the surfactant component. It should be understood that the hydrotrope component is optional and can be omitted if it is not needed for stabilizing the surfactant component. In many cases, it is expected that the hydrotrope component will be present to help stabilize the surfactant component. Examples of the hydrotropes include the sodium, potassium, ammonium and alkanol ammonium salts of xylene, toluene, ethylbenzoate, isopropylbenzene, naphthalene, alkyl naphthalene sulfonates, phosphate esters of alkoxylated alkyl phenols, phosphate esters of alkoxylated alcohols, short chain (C<sub>8</sub> or less) alkyl polyglycoside, sodium, potassium and ammonium salts of the alkyl sarcosinates, salts of cumene sulfonates, amino propionates, diphenyl oxides, and disulfonates. The hydrotropes are useful in maintaining the organic materials, including the surfactant, readily dispersed in the cleaning composition and/or aqueous cleaning solution.

#### Additional Corrosion Inhibitors

Additional corrosion inhibitors which may be optionally added to the detergent compositions of this invention include magnesium and/or zinc. Preferably, the metal ions are provided in water soluble form. Examples of useful water soluble forms of magnesium and zinc ions are the water soluble salts thereof including the chlorides, nitrates and sulfates of the respective metals. If any of the alkalinity providing agents are the alkali metal carbonates, bicarbonates or mixtures of such agents, magnesium oxide can be used to provide the Mg ion. The magnesium oxide is water soluble in such solutions and is a preferred source of Mg ions. In order to maintain the dispersibility of the magnesium and/or zinc corrosion inhibitors in aqueous solution, and in the presence of agents which would otherwise cause precipitation of the zinc or magnesium ions, e.g., carbonates, phosphates, etc., it might be advantageous to include a carboxylated polymer to the solution.

#### Other Additives

The detergent composition can include other additives such as chelating/sequestering agents, bleaching agents, detergent builders or fillers, hardening agents or solubility modifiers, defoamers, anti-redeposition agents, threshold agents, stabilizers, dispersants, enzymes, aesthetic enhancing agents (i.e., dye, perfume), and the like. Adjuvants and other additive ingredients will vary according to the type of composition being manufactured. It should be understood that these additives are optional and need not be included in the cleaning composition. When they are included, they can be included in an amount that provides for the effectiveness of the particular type of component.

Water conditioning polymers can be used as a form of builder. Exemplary water conditioning polymers include polycarboxylates. Exemplary polycarboxylates that can be used as builders and/or water conditioning polymers include those having pendant carboxylate (—CO<sub>2</sub><sup>-</sup>) groups and include, for example, polyacrylic acid, maleic/olefin copolymer, acrylic/maleic copolymer, polymethacrylic acid, acrylic acid-methacrylic acid copolymers, hydrolyzed polyacrylamide, hydrolyzed polymethacrylamide, hydrolyzed polyamide-methacrylamide copolymers, hydrolyzed polyacrylonitrile, hydrolyzed polymethacrylonitrile, hydrolyzed acrylonitrile-methacrylonitrile copolymers, and the like. For a further discussion of chelating agents/sequestrates, see Kirk-Othmer, Encyclopedia of Chemical Technology, Third Edition, volume 5, pages 339-366 and volume 23, pages 319-320, the disclosure of which is incorporated by reference herein.

Bleaching agents for use in a cleaning compositions for lightening or whitening a substrate, include bleaching compounds capable of liberating an active halogen species, such as Cl<sub>2</sub>, Br<sub>2</sub>, —OCl and/or —OBr<sup>-</sup>, under conditions typically encountered during the cleansing process. Suitable bleaching agents for use in the present cleaning compositions include, for example, chlorine-containing compounds such as chlorine, hypochlorite, and/or chloramine. Exemplary halogen-releasing compounds include the alkali metal dichloroisocyanurates, chlorinated trisodium phosphate, the alkali metal hypochlorites, monochloramine and dichloramine, and the like. Encapsulated chlorine sources may also be used to enhance the stability of the chlorine source in the composition (see, for example, U.S. Pat. Nos. 4,618,914 and 4,830,773, the disclosure of which is incorporated by reference herein). A bleaching agent may also be a peroxygen or active oxygen source such as hydrogen peroxide, perborates, sodium carbonate peroxyhydrate, phosphate peroxyhydrates, potassium permonosulfate, and sodium perborate mono and tetrahydrate, with and without activators such as tetraacetylene diamine, and the like. The composition can include an effective amount of a bleaching agent. In a preferred embodiment when the concentrate includes a bleaching agent, it can be included in an amount of about 0.1 wt. % to about 60 wt. %, more preferably between about 1 wt. % and about 20 wt. %, and most preferably between about 3 wt. % and about 8 wt. %.

The composition can include an effective amount of detergent fillers, which does not perform as a cleaning agent per se, but cooperates with the cleaning agent to enhance the overall cleaning capacity of the composition. Examples of detergent fillers suitable for use in the present cleaning compositions include sodium sulfate, sodium chloride, starch, sugars, C<sub>1</sub>-C<sub>10</sub> alkylene glycols such as propylene glycol, and the like. When the concentrate includes a detergent filler, it can be included an amount of about 1 wt. % to about 20 wt. % and between about 3 wt. % to about 15 wt. %.

A defoaming agent for reducing the stability of foam may also be included in the composition to reduce foaming. When the concentrate includes a defoaming agent, the defoaming agent can be provided in an amount of between about 0.01 wt. % and about 3 wt. %.

Examples of defoaming agents that can be used in the composition includes ethylene oxide/propylene block copolymers silicone compounds such as silica dispersed in polydimethylsiloxane, polydimethylsiloxane, and functionalized polydimethylsiloxane such as those available under the name Abil B9952, fatty amides, hydrocarbon waxes, fatty acids, fatty esters, fatty alcohols, fatty acid soaps, ethoxylates, mineral oils, polyethylene glycol esters, alkyl phosphate esters such as monostearyl phosphate, and the like. A

## 11

discussion of defoaming agents may be found, for example, in U.S. Pat. No. 3,048,548 to Martin et al., U.S. Pat. No. 3,334,147 to Brunelle et al., and U.S. Pat. No. 3,442,242 to Rue et al., the disclosures of which are incorporated by reference herein.

The composition can include an anti-redeposition agent for facilitating sustained suspension of soils in a cleaning solution and preventing the removed soils from being redeposited onto the substrate being cleaned. Examples of suitable anti-redeposition agents include fatty acid amides, fluorocarbon surfactants, complex phosphate esters, styrene maleic anhydride copolymers, and cellulosic derivatives such as hydroxyethyl cellulose, hydroxypropyl cellulose, and the like. In a preferred embodiment the anti-redeposition agent, when included in the concentrate, is added in an amount between about 0.5 wt % and about 10% wt %, and more preferably between about 1 wt % and about 5 wt %.

Stabilizing agents that can be used include primary aliphatic amines, betaines, borate, calcium ions, sodium citrate, citric acid, sodium formate, glycerine, maleonic acid, organic diacids, polyols, propylene glycol, and mixtures thereof. The concentrate need not include a stabilizing agent, but when the concentrate includes a stabilizing agent, it can be included in an amount that provides the desired level of stability of the concentrate. In a preferred embodiment the amount of stabilizing agent is about 0 to about 20 wt %, more preferably about 0.5 wt % to about 15 wt %, and most preferably about 2 wt % to about 10 wt %.

Dispersants that can be used in the composition include maleic acid/olefin copolymers, polyacrylic acid, and mixtures thereof. The concentrate need not include a dispersant, but when a dispersant is included it can be included in an amount that provides the desired dispersant properties. Exemplary ranges of the dispersant in the concentrate can be between about 0 and about 20 wt %, more preferably between about 0.5 wt % and about 15 wt %, and most preferably between about 2 wt % and about 9 wt %.

Enzymes can be included in the composition to aid in soil removal of robust soils such as starch, protein, and the like. Exemplary types of enzymes include proteases, alpha-amylases, and mixtures thereof. Exemplary proteases that can be used include those derived from *Bacillus licheniformis*, *Bacillus lemus*, *Bacillus alcalophilus*, and *Bacillus amyloliquefaciens*. Exemplary alpha-amylases include *Bacillus subtilis*, *Bacillus amyloliquefaciens* and *Bacillus licheniformis*. The concentrate need not include an enzyme. When the concentrate includes an enzyme, it can be included in an amount that provides the desired enzymatic activity when the warewashing composition is provided as a use composition. Exemplary ranges of the enzyme in the concentrate include between about 0 and about 15 wt %, more preferably between about 0.5 wt % and about 10 wt %, and most preferably between about 1 wt % and about 5 wt %.

In addition to providing alkalinity and having anti-redeposition properties silicates can also provide further metal protection. Exemplary silicates include sodium silicate and potassium silicate. The detergent composition can be provided without silicates, but when silicates are included, they can be included in amounts that provide for desired metal protection. The concentrate can include silicates in a range between about 10 wt % and about 80 wt %, more preferably between about 30 wt % and about 70 wt %, and most preferably between about 40 wt % and 60 wt %.

The concentrate can include water. In general, it is expected that water may be present as a processing aid and may be removed or become water of hydration. It is expected that water may be present in both the liquid concentrate and in

## 12

the solid concentrate. In the case of the liquid concentrate, it is expected that water will be present in a range of between about 5 wt % and about 95 wt %, more preferably between about 20 wt % and about 75 wt %, and most preferably between about 30 wt % and about 50 wt %. In the case of a solid concentrate, it is expected that the water will be present in ranges between about 5 wt % and about 60 wt %, more preferably between about 15 wt % and about 45 wt %, and most preferably between about 25 wt % and about 40 wt %. It should be additionally appreciated that the water may be provided as deionized water or as softened water.

Various dyes, odorants including perfumes, and other aesthetic enhancing agents can be included in the composition. Dyes may be included to alter the appearance of the composition, as for example, Direct Blue 86 (Miles), Fastusol Blue (Mobay Chemical Corp.), Acid Orange 7 (American Cyanamid), Basic Violet 10 (Sandoz), Acid Yellow 23 (GAF), Acid Yellow 17 (Sigma Chemical), Sap Green (Keystone Analine and Chemical), Metanil Yellow (Keystone Analine and Chemical), Acid Blue 9 (Hilton Davis), Sandolan Blue/Acid Blue 182 (Sandoz), Hisol Fast Red (Capitol Color and Chemical), Fluorescein (Capitol Color and Chemical), Acid Green 25 (Ciba-Geigy), and the like.

Fragrances or perfumes that may be included in the compositions include, for example, terpenoids such as citronellol, aldehydes such as amyl cinnamaldehyde, a jasmine such as C1S-jasmine or jasmal, vanillin, and the like.

The components used to form the detergent can include an aqueous medium such as water as an aid in processing. It is expected that the aqueous medium will help provide the components with a desired viscosity for processing. In addition, it is expected that the aqueous medium may help in the solidification process when is desired to form the concentrate as a solid. When the detergent is provided as a solid, it can be provided in the form of a block, free flowing granular form, powder, or pellet. It is expected that blocks will have a size of at least about 5 grams, and can include a size of greater than about 50 grams. It is expected that the concentrate will include water in an amount between about 1 wt % and about 50 wt %, and more preferably between about 2 wt % and about 40 wt %.

When the components that are processed to form the detergent are processed into a block, it is expected that the components can be processed by extrusion, casting, or pressed solid techniques. In general, when the components are processed by extrusion techniques, it is believed that the composition can include a relatively smaller amount of water as an aid for processing compared with the casting techniques. In general, when preparing the solid by extrusion, it is expected that the composition can contain between about 2 wt % and about 10 wt % water. When preparing the solid by casting, it is expected that the amount of water can be provided in an amount of between about 20 wt % and about 50 wt %.

The detergents of the invention may exist in a use solution or concentrated solution that is in any form including liquid, free flowing granular form, powder, gel, paste, solids, slurry, and foam. The cleaning solutions are suitable to treat any metal surface contaminated with a wide variety of contaminants. Exemplary contaminants include grease, clay, dirt, and oxide by-products. The present solutions may be used by contacting the contaminated metal parts with an effective amount of the aqueous solution. Preferred contact methods include immersion or some type of impingement in which the cleaning solution is circulated or continuously agitated against the metal part or is sprayed thereon. Alternatively, agitation can be provided as ultrasonic waves. The present

13

invention is also suitable for clean-in-place operations that do not require disassembly of equipment.

The warewash detergents of this invention may be used at any temperature, including an elevated temperature of about 90-180° F.

The various forms of the warewashing composition concentrate can be provided in a water soluble packaging film. That is, solids and liquids can be packaged in the water soluble films. Exemplary solids that can be packaged in a water soluble film include powders, pellets, tablets, and blocks. Exemplary liquids that can be packaged in the water soluble film include gels and pastes.

The warewashing composition can be provided in the form of a solid. Exemplary solid dishwashing compositions are disclosed in U.S. Pat. No. 6,410,495 to Lentsch et al., U.S. Pat. No. 6,369,021 to Man et al., U.S. Pat. No. 6,258,765 to Wei et al, U.S. Pat. No. 6,177,392 to Lentsch et al., U.S. Pat. No. 6,164,296 to Lentsch et al., U.S. Pat. No. 6,156,715 to Lentsch et al., and U.S. Pat. No. 6,150,624 to Lentsch et al. The compositions of each of these patents are incorporated herein by reference.

Hard water is often characterized as water containing a total dissolved solids (TDS) content in excess of 200 ppm. This type of water is often referred to as high solids containing water. In certain localities, the water contains a total dissolved solids content in excess of 400 ppm, and even in excess of 800 ppm. The dissolved solids refers to the presence of calcium and magnesium. These components of hard water can be addressed by softening and/or treating the water, using builders, threshold agents, crystal modifiers and/or sequestrants in the detergent composition. In the case of water softening, sodium is often used to displace the calcium and magnesium. The warewashing composition can include builder and/or sequestrant to handle the calcium and thereby reduce its tendency to precipitate with calcium carbonate.

The detergent composition can include an effective amount of anti-etching agent to prevent corrosion to glassware. The calcium that is available in a use composition for precipitating with the aluminum ion can be referred to as "free calcium ion" and is generally considered to be the unchelated calcium ion in the use composition. When the level of free calcium ion is relatively small, it is believed that the weight ratio of the zinc ion to the aluminum ion can be provided at levels that provides the desired corrosion resistances exhibited by a lack of etching. Because the presence of free calcium ion is not a particular concern, it is believed that filming caused by precipitation of calcium ion and aluminum ion will not be very significant. As a result, the ratio of the zinc ion to the aluminum ion can be selected as described in U.S. application Ser. No. 10/612,474 that was filed with the United States Patent and Trademark Office on Jul. 2, 2003, and which is incorporated herein by reference in its entirety. By way of example, the weight ratio of the zinc ion to the aluminum ion can be provided in a range of between about 20:1 to about 1:6, more preferably with a weight ratio of the zinc ion to the aluminum ion in a range of between about 15:1 and about 1:2. In situations where the free calcium ion is available in the use composition at a level sufficient to cause precipitation of the calcium ion and the aluminum ion to provide visible filming, the ratio of the zinc ion to the aluminum ion can be controlled to provide resistance to etching and also resistance to visible filming from precipitation of the calcium ion and the aluminum ion. For example, when the use composition contains in excess of 200 ppm free calcium ion, the weight ratio of the zinc ion to the aluminum ion can be provided at greater than 2:1. By way of an exemplary range, it is believed that the weight ratio of the zinc ion to the aluminum ion can be

14

provided in a range between about 20:1 and about 2:1, more preferably the weight ratio of zinc ion to aluminum ion can be greater than about 3:1, and most preferably can be provided in a range between about 15:1 and about 3:1. In addition, the weight ratio of zinc ion to aluminum ion can be provided at greater than about 4:1 and can be provided at greater than about 6:1. It should be understood that the ratio of zinc ion to aluminum ion may exceed 15:1 and 20:1 when corrosion resistance can still be provided. Furthermore, it should be understood that the reference to the weight ratio of the zinc ion and the aluminum ion refers to a weight ratio based upon the zinc component of the zinc ion and the aluminum component of the aluminum ion. That is, it is the weight of the metal that is determined for purposes of the weight ratio rather than the weight of the entire molecule that may contain the metal. For example, in the case of sodium aluminate, the weight of the aluminum ion refers to the aluminum component of the molecule rather than the entire aluminate ion.

#### Formulating the Detergent Composition

The detergent composition can be formulated to handle the expected corrosion in a given environment. That is, the concentration of the corrosion inhibitor can be adjusted depending upon several factors at the situs of use including, for example, water hardness, soil concentration, alkalinity and the like. In machine warewashing applications, a food soil concentration of about 25 grams per gallon or more is considered high, a concentration of about 15 to about 24 grams per gallon is considered medium, and a concentration of about 14 grams per gallon or less is considered low. Also, water hardness exhibiting 15 grains per gallon or more is considered high, about 6 to about 14 grains per gallon is considered medium, and about 5 grains per gallon or less is considered low. In a use composition, an alkalinity of about 300 ppm or higher is considered high, an alkalinity of about 200 ppm to about 300 ppm is considered medium, and an alkalinity of about 200 ppm or less is considered low. In a use composition, a builder concentration of about 300 ppm or more is considered high, a builder concentration of about 150 ppm to about 300 ppm is considered medium, and a builder concentration of 150 ppm or less is considered low.

Based on the desired minimum concentration of the corrosion inhibitor in the use composition, the amount of the corrosion inhibitor in the concentrate can be calculated knowing the solids content of the use composition and the concentrate can be formulated to provide at least the desired level of corrosion protection.

#### Forming the Concentrate

The components can be mixed/blended, extruded, or cast to form a solid such as pellets, powders or blocks. Heat can be applied from an external source to facilitate processing of the mixture.

A mixing system provides for continuous mixing of the ingredients at high shear to form a substantially homogeneous liquid or semi-solid mixture in which the ingredients are distributed throughout its mass. The mixing system includes means for mixing the ingredients to provide shear effective for maintaining the mixture at a flowable consistency, with a viscosity during processing of about 1,000-1,000,000 cP, preferably about 50,000-200,000 cP. The mixing system can be a continuous flow mixer or a single or twin screw extruder apparatus.

The mixture can be processed at a temperature to maintain the physical and chemical stability of the ingredients, such as at ambient temperatures of about 20-80° C., and about 25-55° C. Although limited external heat may be applied to the mixture, the temperature achieved by the mixture may become elevated during processing due to friction, variances in ambi-

## 15

ent conditions, and/or by an exothermic reaction between ingredients. Optionally, the temperature of the mixture may be increased, for example, at the inlets or outlets of the mixing system.

An ingredient may be in the form of a liquid or a solid such as a dry particulate, and may be added to the mixture separately or as part of a premix with another ingredient, as for example, the corrosion inhibitor component may be separate from the remainder of the detergent. One or more premixes may be added to the mixture.

The ingredients are mixed to form a substantially homogeneous consistency wherein the ingredients are distributed substantially evenly throughout the mass. The mixture can be discharged from the mixing system through a die or other shaping means. The profiled extrudate can be divided into useful sizes with a controlled mass. The extruded solid can be packaged in film. The temperature of the mixture when discharged from the mixing system can be sufficiently low to enable the mixture to be cast or extruded directly into a packaging system without first cooling the mixture. The time between extrusion discharge and packaging can be adjusted to allow the hardening of the detergent block for better handling during further processing and packaging. The mixture at the point of discharge can be about 20-90° C., and about 25-55° C. The composition can be allowed to harden to a solid form that may range from a low density, sponge-like, malleable, caulk consistency to a high density, fused solid, concrete-like block.

Optionally, heating and cooling devices may be mounted adjacent to mixing apparatus to apply or remove heat in order to obtain a desired temperature profile in the mixer. For example, an external source of heat may be applied to one or more barrel sections of the mixer, such as the ingredient inlet section, the final outlet section, and the like, to increase fluidity of the mixture during processing. Preferably, the temperature of the mixture during processing, including at the discharge port, is maintained at about 20-90° C.

When processing of the ingredients is completed, the mixture may be discharged from the mixer through a discharge die. The solidification process may last anywhere from a few minutes to about six hours, depending, for example, on the size of the cast or extruded composition, the ingredients of the composition, the temperature of the composition, and other like factors. Preferably, the cast or extruded composition "sets up" or begins to harden to a solid form within about 1 minute to about 6 hours, more preferably within about 1 minute to about 3 hours, and most preferably within about 1 minute to about 1.0 hours.

The concentrate can be provided in the form of a liquid. Various liquid forms include gels and pastes. Of course, when the concentrate is provided in the form of a liquid, it is not necessary to harden the composition to form a solid. In fact, it is expected that the amount of water in the composition will be sufficient to preclude solidification. In addition, dispersants and other components can be incorporated into the concentrate in order to maintain a desired distribution of components.

The packaging receptacle or container may be rigid or flexible, and composed of any material suitable for containing the compositions produced according to the invention, as for example glass, metal, plastic film or sheet, cardboard, cardboard composites, paper, and the like. The composition is processed at around 150-170° F. and are generally cooled to 100-150° before packaging allowing the mixture to be directly added to the container or other packaging system without structurally damaging the receptacle. As a result, a wider variety of materials may be used as packaging systems.

## 16

The packaging material can be provided as a water soluble packaging material such as a water soluble packaging film. Exemplary water soluble packaging films are disclosed in U.S. Pat. Nos. 6,503,879; 6,228,825; 6,303,553; 6,475,977; and 6,632,785, the disclosures of which are incorporated herein by reference. An exemplary water soluble polymer that can provide a packaging material that can be used to package the concentrate includes polyvinyl alcohol. The packaged concentrate can be provided as unit dose packages or multiple dose packages. In the case of unit dose packages, it is expected that a single packaged unit will be placed in the cleaning apparatus, such as the detergent compartment of the dishwashing machine, and will be used up during a single wash cycle. In the case of a multiple dose package, it is expected that the unit will be placed in a hopper and a stream of water will erode a surface of the concentrate to provide a liquid concentrate that will be introduced into the dishwashing machine.

While the invention is described in the context of a ware-washing composition for washing articles in an automatic dishwashing machine, it should be understood that the composition can be used for washing non-ware items. That is, the composition can be referred to as a cleaning composition and can be used to clean various items and, in particular, items that may suffer from corrosion and/or etching. It should be understood that because the detergent is intended to be used in an automatic dishwashing machine certain components can be excluded from the detergent compositions not intended for use in warewash machines, and vice versa. For example, surfactants that generate a lot of foam may be used in a cleaning composition not intended for use in an automatic dishwashing machine.

Exemplary ranges of the detergent composition in its simplest form include a source of alkalinity and a corrosion inhibitor. It is preferred that the source of alkalinity comprises a range of 30-99 wt. %, more preferably a range of 35-80 wt. % and most preferably a range of 40-70%. The corrosion inhibitor of the invention is present in a preferred range of 1-30 wt. %, a more preferred range of 5-25 wt. %, and a most preferred range of 10 to 20 wt. % of active polymer.

According to the invention, the corrosion inhibitor comprises a synergistic combination of polyacrylic and polymaleic homopolymers. The corrosion inhibitor is primarily comprised of polyacrylic homopolymer. In a preferred embodiment the polyacrylic and polymaleic homopolymers are in a weight percentage ratio of 1:1, in a second, more preferred ratio of 2:1 and in a third, most preferred ratio of 2.33:1 or 7:3.

Exemplary ranges for typical components of detergent compositions including the corrosion inhibitor of the invention are shown in tables 1 and 2. Exemplary ranges when provided as a gel or a paste are shown in Table 1. Exemplary ranges for components of the detergent composition when provided as a solid are shown in Table 2.

TABLE 1

| Component                       | Gel or Paste Warewashing Composition (wt. %) |                  |                 |
|---------------------------------|----------------------------------------------|------------------|-----------------|
|                                 | First Exemplary                              | Second Exemplary | Third Exemplary |
| Water                           | 5-95                                         | 20-75            | 30-50           |
| Silicate/<br>alkaline<br>source | 0-65                                         | 25-60            | 35-55           |

17

TABLE 1-continued

| Gel or Paste Warewashing Composition (wt. %) |                 |                  |                 |
|----------------------------------------------|-----------------|------------------|-----------------|
| Component                                    | First Exemplary | Second Exemplary | Third Exemplary |
| Builder                                      | 0-30            | 3-20             | 6-15            |
| Stabilizer                                   | 0-20            | 0.5-15           | 2-10            |
| Dispersant                                   | 0-20            | 0.5-15           | 2-9             |
| Enzyme                                       | 0-15            | 0.5-10           | 1-5             |
| Polyacrylic-                                 | 0.5-50          | 1-30             | 5-20            |
| Polymaleic                                   |                 |                  |                 |
| Corrosion                                    |                 |                  |                 |
| Inhibitor                                    |                 |                  |                 |
| Surfactant                                   | 0.5-15          | 1-10             | 2-5             |
| Fragrance                                    | 0-10            | 0.01-5           | 0.1-2           |
| Dye                                          | 0-1             | 0.001-0.5        | 0.01-0.25       |

TABLE 2

| Solid Warewashing Composition (wt. %) |                 |                  |                 |
|---------------------------------------|-----------------|------------------|-----------------|
| Component                             | First Exemplary | Second Exemplary | Third Exemplary |
| Water                                 | 5-60            | 15-45            | 25-40           |
| Builder                               | 0-60            | 25-50            | 35-45           |
| Silicate/                             | 0-65            | 25-60            | 35-55           |
| alkaline<br>source                    |                 |                  |                 |
| Dispersant                            | 0-10            | 0.001-5          | 0.01-1          |
| Enzyme                                | 0-15            | 1-10             | 2-5             |
| Polyacrylic-                          | 0.5-50          | 1-30             | 5-20            |
| Polymaleic                            |                 |                  |                 |
| Corrosion                             |                 |                  |                 |
| Inhibitor                             |                 |                  |                 |
| Surfactant                            | 0.5-15          | 1-10             | 2-5             |
| Fragrance                             | 0-10            | 0.01-5           | 0.1-2           |
| Dye                                   | 0-1             | 0.001-0.5        | 0.01-0.25       |

18

The above specification provides a basis for understanding the broad meets and bounds of the invention. The following examples and test data provide an understanding of certain specific embodiments of the invention. The examples are not meant to limit the scope of the invention that has been set forth in the foregoing description. Variations within the concepts of the invention are apparent to those skilled in the art.

## EXAMPLES

### Example 1

According to the invention, several detergent compositions were prepared to deliver various ratios and concentrations of corrosion inhibiting polymer and were compared to a control formulation containing sodium tripolyphosphate as a corrosion inhibitor. The detergent components were kept constant except for the corrosion inhibitor component. Formulas were tested at equal levels of alkalinity (i.e. 2000 ppm of the control and approximately 1000 ppm of the experimentals). To demonstrate synergy four of the eight formulations contain only one component of the corrosion inhibitor (exp #5-8) Whereas the remaining formulas (exp #1-4) contain both components of the corrosion inhibitor. Commercially available polyacrylic acid and maleic acids polymers used in the 8 samples are listed below.

Acusol 929—10,000 MW polyacrylate, 45% active

Acumer 1510—70,000 MW polyacrylate, 25% active

Acusol 445ND—4,500 MW polyacrylate, 95-100% active

Aquatreat AR-6—100,000 MW polyacrylate, 25% active

Belclene 200—400-800 MW polymaleic, 50% active

The components of the test detergents are listed in Tables A and B below.

TABLE A

| CORROSION INHIBITOR COMPONENT |              |                  |                   |                      |              |                  |                   |      |           |
|-------------------------------|--------------|------------------|-------------------|----------------------|--------------|------------------|-------------------|------|-----------|
| Corrosion Inhibitor           | CONTROL      | EXP1             | EXP2              | EXP3                 | EXP4         | EXP5             | EXP6              | EXP7 | EXP8      |
| STPP                          | 25 wt. %     | 0                | 0                 | 0                    | 0            | 0                | 0                 | 0    | 0         |
| PolyAcrylic Acid              | Acusol 445ND | Acusol 929 (45%) | Acumer 1510 (25%) | AquaTreat AR-6 (25%) | Acusol 445ND | Acusol 929 (45%) | Acumer 1510 (25%) |      |           |
| Polymaleic Acid               | 7 wt. %      | 15.5 wt %        | 28 wt. %          | 28 wt. %             | 7 wt. %      | 15.5 wt %        | 28 wt. %          |      |           |
|                               | BELCLENE     | BELCLENE         | BELCLENE          | BELCLENE             | BELCLENE     | 0                | 0                 | 0    | BELCLENE  |
|                               | 200 (50%)    | 200 (50%)        | 200 (50%)         | 200 (50%)            |              |                  |                   |      | 200 (50%) |
|                               | 6 wt. %      | 6 wt. %          | 6 wt. %           | 6 wt. %              |              |                  |                   |      | 6 wt. %   |

TABLE B

## 19

The experimental detergent compositions and the control were tested according to standard protocol in a multi-cycle aluminum corrosion inhibition evaluation for warewash detergents.

A 13"×9" aluminum sheet pan was obtained by cutting a 13"×18" pan in half. The pan was gently cleaned with warm soapy water and a non-abrasive sponge to ensure any foreign materials or residues from cutting and storage were removed. Next a dishwasher was filled with water and heaters were turned on. For high temperature machines, the wash temperature was set to 160° F. and the final rinse temperature was adjusted to 180° F. The Machine was then primed with the desired concentration of detergent and the pan was placed in the second slot from front with the rim facing down and cut edge facing up. The pan rack was then pushed into the machine, the door was closed, and the cycle was started. At the beginning of each cycle, the appropriate amount of detergent was added to the wash tank to make up for the rinse dilution. This was repeated until the desired number of cycles were completed.

## Results:

Pans were rated visually and photographed against a black background. The rating scale used was as follows and was the same for the front and back of each pan:

| Rating | Film                                                               |
|--------|--------------------------------------------------------------------|
| 1      | No corrosion or discoloration                                      |
| 2      | Approximately 25% of the pan is discolored and/or corroded         |
| 3      | Approximately 50% of the pan is discolored and/or corroded         |
| 4      | Approximately 75% of the pan is discolored and/or corroded         |
| 5      | All or nearly all of the pan is heavily discolored and/or corroded |

The results shown in the following table correlate to the compositions shown above. Results are graded visually from 1 (best) to 5 (worst) depending upon the amount of blackening/corrosion of an aluminum pan.

As can be seen, Experiment 8 and Experiment 5 had the highest scores indicating the most corrosion. These experiments represented negative controls and contained either polymaleic or polyacrylic homopolymers as the corrosion inhibitor but not both.

Samples 1, 2, 3, and 4, which had different polyacrylic homopolymer sources combined with polymaleic homopolymer (Belclene 200) all had corrosion inhibition at levels similar to the STPP containing version. The samples also show a synergy that is demonstrated with significantly superior corrosion resistance. This difference in corrosion resistance is not only significantly superior, but is also more than cumulative. As such, the synergistic combination of polyacrylic and polymaleic homopolymers as a corrosion inhibitor represents a biorenewable and environmentally friendly alternative to phosphorus based detergents.

## Example 2

Next, formulations were tested as above for each source of polyacrylic homopolymer with polymaleic homopolymer. Belclene, Acusol 445ND, Acusol 929, Acumer 1510, Aquatreat AR-6 were tested alone at 30 and 70 ppm, and in combination in ratios of 3:7, 5:5 and 7:3. The results indicated that the combination of the two exhibited superior cleaning than either alone, even when the single component was at 100 ppm. Of the combinations, those with at least the same amount of polyacrylic acid to polymaleic acid and preferably a

## 20

higher ratio of polyacrylic acid to polymaleic acid cleaned the best. The best cleaning was observed at 7:3 polyacrylic to polymaleic acid wt. %.

The above specification, examples and data provide a complete description of the manufacture and use of the composition of the invention. Since many embodiments of the invention can be made without departing from the spirit and scope of the invention, the invention resides in the claims hereinafter appended.

## 10 What is claimed is:

1. A warewash detergent composition comprising:
  - (a) an alkaline source in an amount effective to provide a use composition having a pH of at least about 8 and obtained by diluting the detergent composition with water; said alkaline source comprising a silicate present in an amount of from about 35 wt. % to about 55 wt. %;
  - (b) a corrosion inhibitor component in an amount of from about 0.1 wt. % to about 30 wt. % said amount sufficient for reducing corrosion of aluminum or aluminum containing alloys, the corrosion inhibitor component comprising a polyacrylic and a polymaleic homopolymer or their salts in a wt. % ratio of about 7:3 polyacrylic homopolymer to polymaleic homopolymer;
  - (c) a threshold agent in an amount of about 3 wt. % to about 25 wt. %;
  - (d) a surfactant in an amount of from about 1 wt. % to about 5 wt. %;
  - (e) water in an amount from about 10 wt % to about 60 wt. %; and

30 wherein said composition does not include sodium carbonate.

2. The warewash detergent of claim 1 wherein said source of alkalinity further comprises one or more of the following: alkali metal hydroxides, alkali metal salts, phosphates, amines, and mixtures thereof.

3. The source of alkalinity of claim 2 wherein said alkali metal hydroxides include sodium hydroxide, potassium hydroxide, and lithium hydroxide.

4. The source of alkalinity of claim 2 wherein said alkali metal salts include trisodium phosphate, potassium carbonate, and mixtures thereof.

5. The source of alkalinity of claim 1 wherein said silicate includes one or more of sodium metasilicates, sesquisilicates, orthosilicates, potassium silicates, and mixtures thereof.

6. The source of alkalinity of claim 2 wherein said phosphates include sodium pyrophosphate, potassium pyrophosphate, and mixtures thereof.

7. The source of alkalinity of claim 2 wherein said amines include one or more of triethanolamine, monoethanolamine, diethanolamine, and mixtures thereof.

8. The warewash detergent composition according to claim 2, wherein the cleaning agent comprises at least one of an anionic surfactant, a nonionic surfactant, a cationic surfactant, or a zwitterionic surfactant.

9. The warewash detergent composition according to claim 55 1 wherein the detergent comprises less than about 0.1% by weight of phosphorous.

## 10. A detergent composition comprising:

- (a) an alkaline source in an amount effective to provide a use composition having a pH of at least about 8 and obtained by diluting the detergent composition with water; said alkaline source present in an amount of from about 35 wt. % to about 55 wt. %;
- (b) a corrosion inhibitor component in an amount of from about 5 wt. % to about 30 wt. % said amount sufficient for reducing corrosion of aluminum or aluminum containing alloys, the corrosion inhibitor component comprising a combination of polycarboxylic homopolymers

**21**

consisting of a polyacrylic homopolymer and a polymaleic homopolymer or their salts in a wt. % ratio of greater than 1:1 polyacrylic homopolymer to polymaleic homopolymer;

(c) a threshold agent in an amount of about 3 wt. % to about 25 wt. %;

(d) a surfactant in an amount of from about 1 wt. % to about 5 wt. %; and

(e) water in an amount from about 10 wt. % to about 60 wt. %;

wherein said composition does not include sodium carbonate.

**11.** The warewash detergent of claim **10** wherein said source of alkalinity comprises one or more of the following: alkali metal hydroxides, alkali metal salts, metasilicates, phosphates, amines, and mixtures thereof.

**12.** The source of alkalinity of claim **11** wherein said metasilicate includes one or more of sodium metasilicates, sesquisilicates, orthosilicates, potassium silicates, and mixtures thereof.

**13.** The corrosion inhibitor of claim **10** wherein said ratio of polyacrylic homopolymer to polymaleic homopolymer is 2:1.

**14.** The corrosion inhibitor of claim **10** wherein said ratio of polyacrylic homopolymer to polymaleic homopolymer is 7:3.

**15.** The warewash detergent composition according to claim **10**, wherein the cleaning agent comprises at least one of

**22**

an anionic surfactant, a nonionic surfactant, a cationic surfactant, or a zwitterionic surfactant.

**16.** The corrosion inhibitor component according to claim **10**, wherein the corrosion inhibitor component comprises less than about 0.1% by weight of phosphorous.

**17.** A method for cleaning/protecting aluminum or aluminum containing alloys from corrosion comprising:

contacting the surface of the same with a detergent comprising

(a) a corrosion inhibitor comprising a polycarboxylic acid homopolymer selected from the group consisting of: a polyacrylic homopolymer and a poly maleic homopolymer in a wt. % ratio of about 7:3 polyacrylic homopolymer to polymaleic homopolymer; and

(b) a threshold agent in an amount of about 3 wt. % to about 25 wt. % and

wherein said composition does not include sodium carbonate.

**18.** The method of claim **17** wherein said detergent further comprises a metasilicate.

**19.** The method of claim **17** wherein said detergent comprises about 7 wt. % to about 28 wt. % of polyacrylic acid polymer and about 3 wt. and about 12 wt. % of polymaleic polymer.

**20.** The method of claim **17** wherein said detergent composition comprising no more than 55 wt. % of metasilicate.

\* \* \* \* \*

UNITED STATES PATENT AND TRADEMARK OFFICE  
**CERTIFICATE OF CORRECTION**

PATENT NO. : 8,480,808 B2  
APPLICATION NO. : 13/562695  
DATED : July 9, 2013  
INVENTOR(S) : Olson et al.

Page 1 of 1

It is certified that error appears in the above-identified patent and that said Letters Patent is hereby corrected as shown below:

In the Claims:

**Col. 22, Claim 17, Line 12:**

DELETE after a "poly maleic"  
ADD after a --polymaleic--

**Col. 22, Claim 19, Line 22:**

DELETE after about "3 wt."  
ADD after about --3 wt. %--

Signed and Sealed this  
Tenth Day of September, 2013



Teresa Stanek Rea  
*Acting Director of the United States Patent and Trademark Office*